

March 8, 1932.

J. B. HARRIS, JR

1,848,714

COLOR PHOTOGRAPHY

Filed March 5, 1929



INVENTOR

Joseph B. Harris, Jr  
BY  
Lyman E. Dodge  
ATTORNEY

## UNITED STATES PATENT OFFICE

JOSEPH B. HARRIS, JR., OF LOS ANGELES, CALIFORNIA

## COLOR PHOTOGRAPHY

Application filed March 5, 1929. Serial No. 344,185.

This invention relates to color photography, and particularly has reference to the production of a plurality of colored registered images in a single coating on a trans-  
5 parent carrier.

Heretofore quite a few processes have been proposed for forming what is known as a color-photograph, that is, a photograph which exhibits an image of a subject colored 10 corresponding to the coloring of the subject.

Heretofore, it has been proposed to form two registered super-imposed images in the same picture space, one of one color and the other of a substantially complementary color.

15 These colors have been secured usually, one by a toning process and the other by a dyeing process or both by a dyeing process.

A principal object of applicant's invention is to provide a process by which at least two 20 substantially complementary colored super-imposed images, in the same image space, in a single coating, on one side only of a carrier, may be obtained by methods which involve the toning with metallic salts of one image 25 and its subsequent dyeing and the toning of the other image.

Other objects and advantages will appear as the description of a particular manipulation involving the novel features of applicant's invention progresses and the novel features will be particularly pointed out in the appended claims.

In describing the invention in detail and the particular physical product resulting 35 from the application of the process selected to illustrate the invention reference is had to the accompanying drawings wherein has been illustrated a particular physical product resulting from the practice and application 40 of the invention and wherein like characters of reference designate corresponding parts throughout the several views, and in which;

Figure 1, is a schematic representation of a subject; Fig. 2, is a schematic representa-  
45 tion of a red color selection negative repre-

sentative of the reds in the subject, Fig. 1; Fig. 3, is a green color selection negative representative of the green in the subject, Fig. 1; Fig. 4, is a schematic representation of a positive obtained by the use of the negative 50 illustrated by Fig. 2; Fig. 5, is a schematic representation of the positive illustrated by Fig. 4 after having been toned; Fig. 6 is a schematic representation of the positive illustrated by Fig. 5 after printing therein by 55 the negative, Fig. 3, and development; Fig. 7, is a schematic representation of the positive 60 Fig. 6 after being dyed in the toned portions; Fig. 8, is a schematic representation of the positive Fig. 7 after being toned; Fig. 9, is a schematic view illustrating printing from a negative; Fig. 10, is a schematic view illustrating another method of printing from a negative.

Applicant has selected a multi-colored rectangle as a subject by which to illustrate the 65 application of this process. This multi-colored rectangle is illustrated by Fig. 1. It is divided by two diagonal lines forming four triangles. One triangle, 1, is colored red; 70 another 2, is white; another, 3, is colored green, and the fourth, 4, is black.

The first step in carrying out applicant's process is to secure two color selection negatives of the subject, Fig. 1. This is done 75 in the usual and well known manner. The finished red color selection negative is illustrated by Fig. 2. As the red color selection negative, Fig. 2, is a negative made from the subject 1 and in accordance with the usual methods the triangle 1 will be black; the triangle 2 will be black; the triangle 3 will be white; and the triangle 4 will be white.

As the green color selection negative, Fig. 85 3, is a negative of the subject, Fig. 1, and is made in accordance with the usual methods, the triangle 1 will be white; the triangle 2 will be black; the triangle 3 will be black; and the triangle 4 will be white. 90

The first step after obtaining the negatives is to obtain a print of one of them in a photographic emulsion preferably, light sensitive silver salt borne on a transparent carrier. A suitable transparent carrier bearing a suitable photographic emulsion would be the ordinary and well known motion picture film stock. The stock used is illustrated in Fig. 9 in which 5 is the carrier and 6 is the photographic emulsion. Fig. 9 also illustrates the manner in which the print is to be made as 7 designates the carrier of the negative Fig. 2 and 8 designates the image carrying layer thereon. The negative is applied to the back 10 of the carrier and the light 9 is positioned back of the negative. By such an arrangement and by proper regulation of the light value emitted by the light source 9 the image formed in the photograph emulsion will lie 15 substantially adjacent the carrier 5, that is, within the interior of the emulsion 6. A print so made when developed would appear as shown schematically in Fig. 4 in which the triangle 1 would be white; the triangle 2 20 would be white; the triangle 3 black; and the triangle 4 black. The development would be carried out in the usual manner except that at no time must the print be exposed to light. The developer preferably would 25 be one usable in neutral or acid solution such as diamidophenol.

The development should be followed by a short wash and then the print should be immersed for about ten minutes in a bath which 30 consists of:

50 grams sodium citrate  
10 grams copper sulphate  
5 grams potassium ferricyanide  
40 1000 ccs. water

The bath will tone and mordant the print in those portions containing developed silver a sort of red-brown.

The print should next be given a 5 minute 45 wash in water.

Following the wash the print should be immersed in a clearing bath for about ten minutes. A suitable clearing bath would be as follows:

50 12 grams ammonium bromide  
12 grams potassium bichromate  
2 liters water.

The clearing bath acts to restore the sensitivity of the undeveloped light sensitive silver salts which may have been somewhat affected by the previous treatments.

The print is next washed in water for about ten minutes and then dried. The dry print is schematically represented by Fig. 5 in which triangle 1 is white; triangle 2 is white; triangle 3 is red; and triangle 4 is red.

65 The next step is to form an image in the photographic emulsion of the same print as

shown by Fig. 5 by the use of the green color selection negative, Fig. 3. This is done by positioning the negative and print as illustrated by Fig. 10, in which 5 designates the carrier and 6 the photographic emulsion of 70 the print Fig. 5 and 11 designates the carrier and 12 the image carrying layer of the negative, Fig. 3. The position of the printing light is illustrated by 13. By so positioning the negative Fig. 3 in relation to the print Fig. 75 5 as shown in Fig. 10 full advantage will be taken of the undeveloped light sensitive silver salt in the outer portion, that is, the portion remote from the carrier 5 of the photographic emulsion 6. It is of course understood that the negative, Fig. 3, must be so positioned in relation to the print, Fig. 5, that the latent image will be formed in proper registration with the toned and mordanted image already 80 present.

The next operation is to develop. A suitable developer is as follows:

|                          |    |
|--------------------------|----|
| 5 grams diamidophenol    | 90 |
| 50 grams sodium sulphite |    |
| 1 gram potassium bromide |    |
| 5 ccs. lactic acid       |    |
| 1000 ccs. water          |    |

The next operation is to thoroughly wash 95 the film in water and then immerse the film for about 5 minutes in a bath of copper sulphate of a concentration of about 10 grams to 1000 ccs. of water. By this operation the first image, which was somewhat weakened 100 by the action of the second development will be restored.

The result of a second development and the treatment with the copper sulphate bath is to cause the print to appear as shown schematically in Fig. 6 in which triangle 1 is black; triangle 2 is white; triangle 3 is red; and triangle 105 4 is colored with a mixture of both red and black.

After a wash in water for about 10 minutes 110 the print is ready to receive the dye. A suitable dyeing solution is one containing basic dyes and may be made as follows:

|                                       |     |
|---------------------------------------|-----|
| 1 gram auramine, dissolved in alcohol | 115 |
| 2 grams victoria green                |     |
| 2 ccs. acetic acid                    |     |
| 1000 ccs. water                       |     |

The dyeing solution would be allowed to act until the proper color density is obtained 120 which would be about 12 minutes in the usual case.

The next operation is to fix the print. This would be done in a non-acid sodium thiosulfate bath. This bath not only removes all of the undeveloped light sensitive silver salt but also fixes the dye so that the dye is not effected by the long washing in water which then follows.

The appearance of the print after the wash 130 will then be as illustrated by Fig. 7 in which

triangle 1 will be black; triangle 2 will be white; triangle 3 will be green; and the triangle 4 will be colored by a mixture of green and black.

- 5 After the long washing the print is immersed in the copper salt toning bath hereinbefore given. A proper density will be obtained by about ten minutes immersion. After fixing in thiosulphate and a thorough 10 wash in water the film is dried and will appear as shown schematically in Fig. 8 in which the triangle 1 will be red; the triangle 2 will be white; the triangle 3 will be green; and the triangle 4 containing a mixture of 15 both green and red will, by transmitted light, appear black. The colors of the triangles as last described are identical with the similarly positioned triangles in the subject Fig. 1. The operation of the process has resulted 20 in the production of a transparent carrier having a coating on one side only in which in the same picture area two registered superimposed complementary color images have been formed, one a dyed green and the 25 other toned red.

Although applicant has illustrated the principle of his invention by describing the steps of a novel process which result in a novel product, nevertheless, it is to be understood that the particular manipulation described and the product formed does not exhaust the possible manipulation and products lying within the domain of the invention.

What I claim as new and desire to secure 35 by Letters Patent of the United States, is:

1. A photographic process which consists in forming a latent image in a photographic emulsion, developing, toning with a copper salt and after clearing with a bath of ammonium bromide and potassium bichromate in water solution forming another latent image in the same photographic emulsion, developing and then dyeing the toned image in a water solution of a basic dye, then after 45 fixing, toning the second formed image with a copper salt.

2. A photographic process which consists in forming a metallic image in a photographic emulsion, toning said image and clearing 50 with a bath of ammonium bromide and potassium bichromate in water solution and thereafter forming a latent image in the said photographic emulsion, developing and fixing said last mentioned image, and after dyeing the first mentioned image with a basic dye toning the last mentioned image.

3. The process which consists in first forming a silver image in a photographic emulsion, then toning with a copper salt that image substantially a red-brown, then forming another silver image in the same photographic emulsion, then green dyeing the first mentioned image with a basic dye, fixing, 65 and then red toning the second mentioned

image without affecting the color of the first image.

4. A photographic process which consists in forming a latent image in a photographic emulsion, developing, toning with a metallic 70 salt and after clearing with a bath of ammonium bromide and potassium bichromate in water solution, forming another latent image, in the same photographic emulsion, developing and then dyeing the toned image 75 in a water solution of a basic dye, then after fixing, toning the second formed image with a metallic salt.

JOSEPH B. HARRIS, JR.

80

85

90

95

100

105

110

115

120

125

130